

H. C. HARRISON.

FERROSILICON ALLOYS OF A DEFINITE COMPOSITION.

APPLICATION FILED DEC. 14, 1909. RENEWED SEPT. 17, 1914.

1,134,129.

Patented Apr. 6, 1915.



FIG. 1. SOLUBILITY % OF ALLOY IN HCl



Inventor

Witnesses

Geo. A. Sykes,  
B. B. Bellings.

FIG. 2.

H. C. Harrison  
Witnesses Fisher &  
Witnesses, from  
Attorney

# UNITED STATES PATENT OFFICE.

HERBERT CHAMPION HARRISON, OF LOCKPORT, NEW YORK, ASSIGNOR, BY MESNE ASSIGNMENTS, TO ELECTRO METALLURGICAL COMPANY, A CORPORATION OF WEST VIRGINIA.

## FERROSILICON ALLOYS OF A DEFINITE COMPOSITION.

1,134,129.

Specification of Letters Patent. Patented Apr. 6, 1915.

Application filed December 14, 1909, Serial No. 533,110. Renewed September 17, 1914. Serial No. 862,256.

To all whom it may concern:

Be it known that I, HERBERT CHAMPION HARRISON, a subject of the King of Great Britain, residing at Lockport, Niagara county, and State of New York, have invented certain new and useful Improvements in Ferrosilicon Alloys of a Definite Composition; and I do hereby declare the following to be a full, clear, and exact description of the invention, such as will enable others skilled in the art to which it appertains to make and use the same.

This invention relates to ferrosilicon alloys and has for its object to produce products of such a nature as will enable the user to attain more uniform results than heretofore.

With these ends in view the invention consists in the series of definite alloys more fully hereinafter disclosed and particularly pointed out in the claims.

Referring to the accompanying drawings forming a part of this specification: Figure 1 is a diagram showing solubility curves for ferrosilicon alloys from zero to 54 per cent. silicon content. Fig. 2 is a diagram illustrating the relative freezing and melting points of the various alloys of from 33 per cent. silicon to 54 per cent. silicon.

It is well known that the chemical compound FeSi exists, and I have shown in my pending application #510,477 filed July 30, 1909, for ferrosilicon products and methods of producing the same that the compound  $Fe_3Si_7$  exists; and therefore in an alloy consisting of iron and silicon between the limits of pure iron and no silicon, and pure silicon and no iron we have these two compounds. I have now demonstrated that in the series Fe; FeSi;  $Fe_3Si_7$ ; and Si that any two of these members when taken consecutively will when liquid dissolve into each other in all proportions, but when just solid, each is mutually insoluble in the other.

That is to say, I have proved that Fe and FeSi when liquid are mutually soluble in all proportions; that FeSi and  $Fe_3Si_7$  are the same; and that  $Fe_3Si_7$  and Si are likewise mutually soluble. I have also proved that when Fe and FeSi are just solid, or when FeSi and  $Fe_3Si_7$ , or when  $Fe_3Si_7$  and Si, are just solid, they are mutually insoluble. Throughout this specification the sym-

bols Fe and Si are used to indicate metallic iron and metallic silicon respectively.

It follows from the foregoing that all the alloys between Fe and FeSi consist of solid mixtures of Fe and FeSi in varying proportions. And from the well known theory of eutectics as set forth in *Metallic Alloys* by G. H. Gulliver, 1908, and in other publications it follows that between these limits a eutectic will exist corresponding to a formula  $Fe_3Si$ , which itself consists of a solid crystal of pure FeSi, and a crystal of pure iron. This enables one to foretell with a great deal of certainty the exact constitution of all alloys between the above limits. That is to say, on cooling an alloy from the liquid state which lies between the limits of this eutectic and pure iron, the pure iron in excess will crystallize out first until the remainder reaches the composition of the eutectic, when without a further drop in temperature which now remains constant the eutectic will crystallize out until the whole mass is solid. The line AE<sub>1</sub> in Fig. 2 represents the freezing points and compositions of the various alloys that may exist between pure iron and the eutectic  $Fe_3Si_1$ ; the point E<sub>1</sub> corresponding to the compositions of this eutectic and also to its freezing point. And again, on cooling an alloy which lies between the limits of the eutectic and FeSi, first, that FeSi which is an excess will crystallize out until the composition of the remainder reaches the composition of the eutectic. Thereupon this eutectic will crystallize out at a constant temperature until the whole mass is solid. The line E<sub>1</sub>B also represents the freezing points and compositions of the various alloys that may exist between the eutectic  $Fe_3Si$  and FeSi while the point B corresponds to the composition and freezing point of the compound FeSi.

I have discovered that in this series of alloys neither  $Fe_3Si_7$  nor free silicon can exist as such. I have been enabled to prove this by dissolving all the iron in these alloys in hydrochloric acid and determining the silicon in the residue, which silicon in said residue was found to exist in the form of silicia. Had it existed as silicon in the original alloy it would have been unattacked and would have been weighed as silicon instead of silica. In the same way had  $Fe_3Si_7$

been present in these alloys all of the iron would not have been soluble in the hydrochloric acid since this compound I have demonstrated to be insoluble in that reagent. 5 By the same procedure I have demonstrated that all the alloys between  $Fe_3Si_7$  and  $Fe_3Si_8$  consists of solid mixtures of pure  $Fe_3Si_7$  and pure  $Fe_3Si_8$  in varying proportions. And I have found that a second eutectic corresponding to  $Fe_3Si_8$  which is itself a crystal of  $Fe_3Si_7$  together with a crystal of  $Fe_3Si_8$ , exists. Upon cooling an alloy from the liquid existing between the limits  $Fe_3Si_7$  and  $Fe_3Si_8$ , the  $Fe_3Si_7$  in excess crystallizes out 10 first until the composition of the remainder reaches that of the second eutectic when at a constant temperature the latter will crystallize out until the mass is solid. The line  $BE_2$ , in like manner represents the freezing points 15 and the compositions of these various latter alloys. Also upon cooling an alloy between the limits of the second eutectic and  $Fe_3Si_7$ , that  $Fe_3Si_7$  which is in excess will crystallize out first, and until the composition of 20 the remainder reaches that of the second eutectic, when at a constant temperature this latter will crystallize out until the whole mass is solid. The line  $E_2C$  represents the compositions and freezing points of these 25 said alloys.

In this series of alloys neither free iron nor free silicon exists; and I have proved this by showing that when any such alloys are treated with hydrochloric acid the iron 30 which is dissolved out together with the residue which is left, adds up to considerably more than 100 per cent. and that in every case the excess of weight of the residue, which consists of silica and  $Fe_3Si_7$ , is 35 due to the fact that the silicon which was combined with the iron dissolved is weighed in the said residue as silica and not silicon. On the other hand the actual amount of 40 silicon in the silicia is found in every case to be that amount which would have combined with the dissolved iron as  $Fe_3Si_7$ ; thus proving that no free iron was present. Furthermore upon subtracting the silica from the residue a compound is left corresponding 45 to  $Fe_3Si_7$ , thus showing that there was no free silicon present.

In addition to the above it is well known that free silicon changes the color of the alloy, and in the case above no such color 50 changes appear up to the limit of  $Fe_3Si_7$ . By a like procedure I found that between the limits  $Fe_3Si_7$  and Si, all alloys consist of solid mixtures of pure  $Fe_3Si_7$  with pure Si; and that a eutectic exists corresponding 55 to  $Fe_3Si_7$  which is itself composed of a crystal of  $Fe_3Si_7$  and a crystal of silicon. Upon cooling such an alloy from the liquid state between the limits of  $Fe_3Si_7$  and  $Fe_3Si_8$ , that  $Fe_3Si_7$  which is in excess will first crystallize 60 out until the remainder reaches the composi-

tion corresponding to the third eutectic, whereupon this latter will crystallize out at a constant temperature until the whole mass is solid. The line  $CE_3$  represents the compositions and freezing points of these last 70 mentioned alloys. Upon cooling an alloy between the limits of the third eutectic corresponding to  $Fe_3Si_9$  and Si, that silicon which is in excess will crystallize out until the remainder reaches the composition of the 75 third eutectic when this will crystallize out at a constant temperature until the whole mass is solid. The line  $E_3D$  represents the compositions and freezing points of these 80 alloys. In this last series of alloys I have also discovered that neither free iron nor free  $Fe_3Si_7$  exists as the whole of the product is insoluble in hydrochloric acid. The foregoing results may be graphically illustrated as in Fig. 1, wherein the line 1 represents a 85 solubility curve which passes through a series of seven illustrative determinations that were actually carried out. In this figure the percentages of silicon are plotted vertically and the percentages of solubilities in 90 hydrochloric acid of the alloys illustrated are plotted horizontally. The solubility of  $Fe_3Si_7$  is 66.2 per cent. because all its iron is soluble whereas the solubility of  $Fe_3Si_8$  is zero, because none of its iron is soluble; and 95 these two compounds mark the extremities of line 1. The other alloys illustrated in Fig. 1 have solubilities corresponding to their positions on said line. These determinations of solubilities in hydrochloric acid 100 show that the solubilities found to actually exist in practice in the case of alloys varying between 37.24 per cent. and 54 per cent. silicon content agree closely with what would be necessary if all alloys between 33 per 105 cent. and 54 per cent. of silicon consisted of solid mixtures of  $Fe_3Si_7$  and  $Fe_3Si_8$ . And in no case do these determinations agree with an assumption that the alloys consist of any other constitution, for if they did 110 these would fall on one or the other of the hypothetical curves 2, 3 and 4. The line 2 represents the solubilities of mixtures of  $Fe_3Si_7$  with the hypothetical  $Fe_2Si_3$ ; the line 3 represents mixtures of  $Fe_3Si_7$  with either 115 the hypothetical  $Fe_3Si_2$  or the hypothetical  $Fe_3Si_1$ ; and the line 4 represents mixtures of  $Fe_3Si_7$  with Fe. Since no determinations lie on or near any of the lines other than line 1, and all of them lie on line 1, the figure 120 represents graphically the foregoing results.

The foregoing information lays bare the 125 constitutions and compositions of the whole range of alloys, and enables one to produce at will by following the procedure below not only any particular alloy of an unvarying character, but a whole series of alloys which will always behave the same when steel is treated therewith.

In order to produce an alloy which will be 130

uniform in its behavior and unvarying in its composition, I chemically proportion the charge to produce the alloy in question; I provide sufficient carbon to effect a theoretical reduction of the silica together with such an excess of carbon as may be found desirable from practical considerations; I apportion the input of power to the furnace to the size of the furnace operated and in

such manner as to insure a practically theoretical yield of the alloy sought from the charge material, all as fully set forth in connection with the manufacture of  $Fe_3Si$ , in my copending application #530,787 filed

December 1, 1909.

The advantages to the steel maker in using a series of unvarying and constant alloys resides in the fact that he knows beforehand how the silicon is combined with the iron in the alloy and therefore he knows just how the alloys will behave in the molten metal when employing different temperatures, which is not the case at present. He knows the temperature to which the steel must be raised to melt the alloy and therefore he knows that a higher temperature must be employed to chemically break up the alloy in the metal. He knows whether it will be endothermic or exothermic in the melt, and therefore whether it will chill or heat the metal. In fact, after the steel maker has once attained perfection with a definite

alloy, he can be assured of indefinitely repeating his success which is not the case at present.

35

Of course it is evident to those skilled in the art that the foregoing principles are applicable to alloys in general, and therefore I do not wish to be limited to any specific alloys except as may be required by the 40 claims.

What I claim is:—

1. The herein described ferro alloy having a definite composition and a definite constitution, comprising solid mixtures of 45 definite chemical compounds containing iron, substantially as described.

2. The herein described ferro alloy having a definite composition and a definite constitution, comprising solid mixtures of 50 definite chemical compounds containing iron and silicon, substantially as described.

3. The herein described ferro alloy having a definite composition and a definite constitution consisting of a plurality of definite 55 chemical compounds of iron and silicon, substantially as described.

In testimony whereof, I affix my signature, in presence of two witnesses.

HERBERT C. HARRISON.

Witnesses:

T. A. WITHERSPOON,  
J. FRED KELLEY.